

1

2,733,235

## MINERAL OIL ADDITIVE

Thomas Cross, Jr., Union, and Jeffrey H. Bartlett, Westfield, N. J., assignors to Esso Research and Engineering Company, a corporation of Delaware

No Drawing. Application February 6, 1952,  
Serial No. 270,293

16 Claims. (Cl. 260—125)

This invention relates to mineral oil compositions and particularly to lubricating oils in which an additive has been incorporated to improve the properties of the same.

Modern developments in the design of internal combustion engines, with increasing engine speeds and compression ratios, have imposed a severe strain on the lubricants employed. In particular, the crankcase oil is raised to a high temperature and in the course of its circulation through the engine is rapidly exposed to air under conditions highly conducive to destructive oxidation. Oxidative breakdown of the oil results in the formation of acidic products which corrode bearing surfaces and do considerable harm to the engine generally. Furthermore, the metallic corrosion products have the effect of catalyzing further oxidative breakdown of the oil.

It is also known that in modern internal combustion engines, such as aviation gasoline engines operating at relatively high temperatures due to their high power output, or in high speed diesel engines due to incomplete combustion, piston rings have a tendency to become stuck in grooves. Lacquer and carbon formation appear to be the principal reasons for this occurrence. Moreover, scuffing of top lands due to the formation of hard carbon, particularly when using high viscosity index oils, may cause serious damage to the engine.

It has been found, in accordance with the present invention, that destructive oxidation of lubricating oils and deposition of carbon and lacquer may both be substantially reduced by the addition to the oil of a small amount of a new additive. This additive may be described as a reaction product obtained by reacting a sulfide of phosphorus or other combinations of the elements sulfur and phosphorus with an aliphatic alcohol ester of an alkenyl succinic acid containing a single alkenyl group of 4 to 24 carbon atoms. The ester may be a diester, a half ester, or a group I or II metal salt of a partial ester. Metal salts of the phospho-sulfurized reaction products, when the metal is selected from the metals of group I or II of the periodic table, may also be employed to advantage, especially when the detergent effects of the additive are to be emphasized. These additives have the effect of reducing oxidation and the formation of carbon deposits or sludge in lubricating oils. They are also sometimes useful, when added to lubricants, for protecting metallic surfaces of such engines against corrosion. The additives are also useful generally as anti-oxidants in mineral oil products of all types.

The alkenyl succinic acid used to form the esters may be conveniently prepared by condensing mono-olefins with maleic acid or maleic anhydride, employing an elevated temperature, for example 160° C. or higher. The condensation process results in the formation of an alkenyl substituted succinic acid or anhydride. A typical reaction follows:

2



For introducing the alkenyl groups desired in accordance with the present invention, any mono-olefin having from 4 to 24 carbon atoms, preferably 6 to 16 carbon atoms, may be employed. Such olefins include normal and branched chain olefins and polymers of the same, as well as mixtures of olefins occurring in technical products. Examples of suitable olefins include n-butylene, iso-butylene, 2-ethyl-1-butene, diamylene, 1-decene, 1-tetradecene, 1-octadecene, 6-24 polypropylenes, C<sub>16</sub>-C<sub>18</sub> olefins from the Fischer synthesis, C<sub>24</sub> dechlorinated wax, cracked gasoline, and similar products. The preparation of alkenyl succinic acids and the like is well known to the art.

The alkenyl substituted acids or anhydrides of the type described above may be esterified by reaction with a saturated or unsaturated aliphatic alcohol, employing the usual esterification methods, preferably with the aid of an esterification catalyst such as p-toluene sulfonic acid and a water entraining agent. Typical examples of suitable alcohols which may be employed are the following:

Methyl alcohol  
Ethyl alcohol  
Allyl alcohol  
n-Propyl alcohol  
n-Butyl alcohol  
Isobutyl alcohol  
n-Amyl alcohol  
Isoamyl alcohol  
35 Allyldiethylcarbinol  
n-Octyl alcohol  
2-ethylhexyl alcohol  
Cetyl alcohol  
Oleyl alcohol  
40 Isodecyl "Oxo" alcohol  
Iso tridecyl "Oxo" alcohol  
Iso hexadecyl "Oxo" alcohol.

A group of alcohols especially adapted for use in connection with the present invention are the so-called "Oxo" alcohols. These alcohols are prepared by the reaction of carbon monoxide and hydrogen with olefins obtainable from petroleum products followed by hydrogenation of the resulting aldehydes. Materials such as di-isobutylene and C<sub>7</sub> olefins are suitable for this purpose; also higher molecular weight olefinic materials are sometimes employed. The alcohols obtained in this manner are primary alcohols and normally have a highly branched chain structure. Preferably, primary monohydric aliphatic alcohols having in the range of 1 to 30 carbon atoms per molecule and containing no more than one olefinic double bond are used. Particularly preferred alcohols are those having 6 to 20 carbon atoms.

The alkenyl succinic acid or anhydride may be partially or completely esterified with one or more alcohols of the above mentioned type. The half ester may be converted into a metal salt by reaction with a hydroxide, carbonate or other basic reacting compound of a metal of group I or II of the periodic table. Such metals include sodium, potassium, calcium, strontium, barium, etc. although barium salts are particularly preferred. This reaction may be conducted at a temperature in the range of about 50° to 400° F.

Specifically, the esters to be reacted with the reactive sulfur- and phosphorus-containing material have the following formula:



wherein R is an alkenyl radical having 4 to 24 carbon atoms, R' is selected from the group consisting of alkyl and alkenyl radicals having 1 to 30 carbon atoms, M is selected from the group consisting of R', group I and II metals and hydrogen, and n is 1 to 2. The integer n will be 2 when a divalent metal salt is prepared.

The esters or ester salts derived from the alcohols and alkenyl succinic acids described above are then reacted with a reactive sulfur and phosphorus-containing material. It is preferable to employ a sulfide of phosphorus, such as  $\text{P}_2\text{S}_3$ ,  $\text{P}_2\text{S}_5$ ,  $\text{P}_4\text{S}_3$ , or  $\text{P}_4\text{S}_7$ , or mixtures thereof. Mixtures of elemental sulfur and elemental phosphorus may likewise be employed, in which case it is preferable to employ powdered sulfur and white phosphorus. Likewise, a mixture of one or more sulfides of phosphorus and elemental sulfur and/or elemental phosphorus may be employed. The amounts of sulfur and phosphorus which are advantageously employed depend upon such factors as the number of double bonds present in the ester in double-bonded hydrocarbon groups, and the ultimate phosphorus and sulfur content desired in the product. For example, about 0.2 to 1.5 mols of a sulfide of phosphorus may be used for each mol of ester or ester salt. It is generally preferred to react from 0.1 to 1 atom of phosphorus and 0.1 to 3 atoms of sulfur for each such double-bond in the ester molecule. About one-half mol of sulfide of phosphorus, such as  $\text{P}_2\text{S}_5$ , is preferably used for each mol of double bond. In general, the temperature at which the reaction of the sulfide of phosphorus or mixture of sulfur and phosphorus with the ester is carried out is in the range of about 200° to 500° F., preferably about 250°-400° F., and the time required to substantially complete the reaction is generally from 1 to 10 hours. Usually, at least about 0.3 to 0.5 weight percent of both sulfur and phosphorus should be introduced into the product.

It is generally desirable to employ an organic solvent during the reaction. The solvent should be relatively inert to phosphorus and sulfur. Such solvents include, for example, benzene, o-dichlor-benzene, lubricating oil base stocks, and the like. In preparing an additive for use in a mineral oil, it is usually convenient to employ a mineral oil as the medium for the reaction, and thus prepare a concentrate for convenient use in blending with the oil.

As stated above, the phospho-sulfurized reaction products prepared as described may be used as such or in the form of their group I or II metal salts. The metals employed are preferably group II metals and the barium salts are particularly desirable and convenient to prepare. Such metal salts may be prepared by reacting the phosphorus and sulfur-containing reaction product with metallic oxides or hydroxides or other basic reacting compounds of such metals. The metallic compounds may be added to the reaction mixture in which the phosphorus and sulfur-containing reaction products are formed, and the mixture heated to a temperature of the range of 50°-400° F. Sufficient basic reacting metallic compound may be used to neutralize the phospho-sulfurized ester.

The additives of the present invention are preferably added to mineral oils in proportions ranging from 0.01% to 15%, the proportion being preferably about 1.0 to 5.0% when employed as corrosion inhibitors and detergents in mineral lubricating oils. The proportions giving

the best results will vary somewhat according to the nature of the additive and the specific quality characteristics of the oil to be improved by the use of the additive. For commercial purposes, when the additives are to be employed in mineral lubricating oils, it is convenient to prepare concentrated oil solutions in which the amount of additive in the compositions ranges from about 20 to 50% by weight, and to transport and store them in such form. In preparing lubricating oil compositions for use as crankcase lubricants, the additive concentrate is merely blended with the base oil in the required amount.

Below are given detailed descriptions of preparations of several examples of mineral oil additives of the type described above as well as various laboratory tests which were applied to determine their effectiveness when employed in lubricating oil compositions. It is to be understood that these examples are given to illustrate the present invention and are not to be construed as limiting the scope thereof in any way.

#### Example 1

*Product A.*—The "Lorol B" half ester of  $\text{C}_{10}-\text{C}_{12}$  alkenyl succinic acid having a neutralization number of 116 was prepared by partially esterifying  $\text{C}_{10}-\text{C}_{12}$  alkenyl succinic acid with "Lorol B" alcohol (a mixture of  $\text{C}_{10}-\text{C}_{18}$  alcohols having an average molecular weight of 207). 250 grams of the half ester were placed in a 1-liter flask and neutralized with a solution containing 82 g. barium hydroxide and 150 g.  $\text{H}_2\text{O}$ . The water was removed by heating. A 20% concentration of the resulting barium salt of the half ester in a lubricant having an S. S. U. viscosity at 210° F. of about 50 was then prepared. The concentrate (Product A) had a neutralization number (mg. KOH per gram of product) of 6.6.

*Product B.*—500 g. of Product A (containing about 0.1 mol of the barium salt of the half ester) was heated to 250° F. and 11.1 g. (about 0.05 mol) of  $\text{P}_2\text{S}_5$  were slowly added over a period of one hour with rapid stirring. The temperature was then raised to 300° F. and kept at that temperature for two hours. The reddish-brown product was then filtered through "Hy-flo" diatomaceous filter acid and analyzed:

|                    | Weight Percent |
|--------------------|----------------|
| Ash                | 3.88           |
| Barium             | 2.26           |
| Phosphorus         | 0.60           |
| Sulfur             | 1.19           |
| Neutralization No. | 9.49           |

#### Example 2.—Carbon black dispersion test

This test is used to measure the dispersive power of the lubricating oils. 500 cc. of a 1% blend of Product B in a solvent-extracted Mid-Continent praffinic base oil of 52 seconds viscosity (Saybolt) at 210° F. was agitated with 6% by weight of carbon black and allowed to settle for 24 hours at a temperature of 200° F. For comparison, a similar amount of base oil was similarly treated. The test was applied to the Product B. The results are shown in Table I.

TABLE I

|    | Oil                                                                                                   | Observation after 24 Hours |                    |
|----|-------------------------------------------------------------------------------------------------------|----------------------------|--------------------|
|    |                                                                                                       | Ces. of Clear Oil          | Ces. of Dispersion |
| 70 | Base Oil                                                                                              | 169                        | 340                |
|    | Base Oil + 1% Barium "Lorol B" alkenyl succinate- $\text{P}_2\text{S}_5$ reaction product (Product B) | 0                          | 500                |

It is seen that the metal salt of the half ester imparted dispersive properties to the oil containing it.

*Example 3.—Indiana oxidation test*

In this test a glass plate is inserted in the test oil and the weight of the varnish film deposited on the plate during 48 hours is measured. The oil during the test is held at about 341° F., and air is passed through the oil at the rate of 10 liters per hour. This test was applied to a base oil consisting of a solvent extracted Mid-Continent oil of S. A. E.-20 grade and to a blend of this oil and 1.0% of Product B. The results are shown in Table II:

TABLE II

| Oil                     | Varnish on Glass Plate (mg.) |
|-------------------------|------------------------------|
| Base oil                | 3.0                          |
| Base Oil+1.0% Product B | 0.5                          |

This test reveals the detergency characteristics of additives added to oils, the degree of detergency generally being inversely proportional to the amount of varnish deposited on the glass plate. The product of the present invention effected a substantial improvement in the detergency characteristics of the oil containing it.

*Example 4.—Laboratory bearing corrosion test*

A blend was made containing 1% of Product B in a lubricating oil base consisting of a well refined, solvent extracted paraffinic mineral lubricating oil of S. A. E. 20 viscosity grade. This blend and a sample of the unblended base oil were submitted to a corrosion test designed to test the effectiveness of the additive in inhibiting corrosion of a typical copper-lead bearing.

In this test 500 cc. of the oil were placed in a glass oxidation tube (13 inches long and 2½ inches in diameter) fitted at the bottom with a ¼ inch air inlet tube perforated to facilitate air distribution. The oxidation tube was then immersed in a heating bath so that the oil temperature was maintained at 325° F. during the test. Two quarter sections of automotive bearings of copper-lead alloy of known weight having a total area of 25

mg. in weight, determined by interpolation of the data obtained in the various periods.

TABLE III

| 5  | Oil Tested                              | Bearing Corrosion Life, (Hours) |
|----|-----------------------------------------|---------------------------------|
| 10 | Base Oil                                | 13                              |
| 10 | Base Oil plus 1.0 Wt. Percent Product B | 37                              |

The oil containing Product B showed a much greater resistance to corrosion of the metal than the uncompounded base oil.

*Example 5*

A series of preparations were carried out in which C<sub>10</sub>-C<sub>12</sub> alkenyl succinic acid and C<sub>8</sub>-C<sub>10</sub> alkenyl succinic acid were esterified with various saturated and unsaturated aliphatic alcohols. The resulting esters were then directly phosphosulfurized with phosphorus pentasulfide.

Product C was prepared in the following manner. A 1-liter, 4-neck flask equipped with a stirrer, thermometer, nitrogen inlet tube and gas exit tube was charged with 100 g. of the C<sub>13</sub> "Oxo" ester of C<sub>10</sub>-C<sub>12</sub> alkenyl succinic acid and 176.5 g. of a phenol extracted Mid-Continent distillate of 45.1 seconds (Saybolt) viscosity at 210° F. After heating the mixture to 250° F., 17.5 g. of P<sub>2</sub>S<sub>5</sub> was added during 5 minutes and heating was continued to 300° F., at which temperature it was maintained for 4 hours. A slow stream of nitrogen was passed thru the mixture throughout the course of the reaction. The product was filtered while hot with "Hy-flo" leaving 15 g. of resinous material on the flask. Oil concentrate (Product C) contained about 40% active ingredient.

Products D through G were prepared substantially in accordance with the procedure employed in making Product C. Table IV, below, presents information on the properties of the esters, the molar ratio of ester to P<sub>2</sub>S<sub>5</sub> used in the phosphosulfurization reaction and the analysis of the resulting products. In each case, the product contained about 40% by weight of active ingredient in oil.

TABLE IV

| Product | Ester Treated                                                                          | Properties of Ester    |                       | Molar Ratio, Ester/P <sub>2</sub> S <sub>5</sub> | Analyses of Product, Weight Percent |        |
|---------|----------------------------------------------------------------------------------------|------------------------|-----------------------|--------------------------------------------------|-------------------------------------|--------|
|         |                                                                                        | Neut. No. <sup>1</sup> | Sap. No. <sup>2</sup> |                                                  | Phosphorus                          | Sulfur |
| C-----  | C <sub>10</sub> "Oxo" ester of C <sub>10</sub> -C <sub>12</sub> alkenyl succinic acid. | 3.4                    | 203                   | 2/1                                              | 0.53                                | 3.71   |
| D-----  | C <sub>10</sub> "Oxo" ester of C <sub>10</sub> -C <sub>12</sub> alkenyl succinic acid. | 3.4                    | 112                   | 2/1                                              | 0.50                                | 3.60   |
| E-----  | "Lorol B" ester of C <sub>10</sub> -C <sub>12</sub> alkenyl succinic acid.             | 5.6                    | 181                   | 2/1                                              | 0.38                                | 3.37   |
| F-----  | Oleyl ester of C <sub>10</sub> -C <sub>12</sub> alkenyl succinic acid.                 | 1.1                    | 112                   | 2/1                                              | 1.34                                | 3.27   |
| G-----  | n-decyl ester of C <sub>8</sub> -C <sub>10</sub> alkenyl succinic acid.                | 1.1                    | 203                   | 2.7/1                                            | 0.51                                | 3.75   |

<sup>1</sup> Neutralization number, mg. KOH/g. ester.

<sup>2</sup> Saponification number, mg. KOH/g. ester.

square centimeters were attached to opposite sides of a stainless steel rod which was then immersed in the test oil and rotated at 600 R. P. M., thus providing sufficient agitation of the sample during the test. Air was then blown through the oil at a rate of 2 cubic feet per hour. At the end of each 4-hour period the bearings were removed, washed with naphtha, and weighed to determine the amount of loss by corrosion. The bearings were then repolished (to increase the severity of the test), reweighed, and then subjected to the test for additional 4-hour periods in like manner. The results are given in Table III, below, as "corrosion life," which indicates the number of hours required for the bearings to lose 100

65 The above products were tested by the copper corrosion test which is a modification of the C. R. C. method, L-16-445. Blends were prepared containing 0.5% by weight of each of the active ingredients (Products B-G) in a solvent extracted Mid-Continent base oil having 48.3 seconds (Saybolt) viscosity at 210° F. A polished metallic copper strip was immersed in each blend and in a sample of the base oil for a period of one-half and three hours at 210° F. The extent of staining on each strip was then rated on a scale of from "1" (no stain) to "10" (black surface film). The results of these 70 tests are given in Table V, below:

7  
TABLE V

| Product in Base Oil      | Copper Corrosion Rating |         |
|--------------------------|-------------------------|---------|
|                          | 1/2 Hour                | 3 Hours |
| None (base oil alone) .. | 3                       | 5       |
| B ..                     | 3                       | 6       |
| C ..                     | 2                       | 2       |
| D ..                     | 2                       | 10      |
| E ..                     | 2                       | 3       |
| F ..                     | 2                       | 3       |
| G ..                     | 2                       | 2       |

The phospho-sulfurized esters reduced the corrosiveness of the oil containing them. The phospho-sulfurized metal salt of the ester (Product B) had substantially no effect.

The above products were also evaluated by the laboratory corrosion test described in Example 4. In this case, the blends tested were prepared by dissolving 0.5% by weight of the active ingredient of each of the products in a white oil having a viscosity at 210° F. of 54.2 seconds (Saybolt). The white oil was a relatively unstable product obtained by successive treatment of a solvent extracted coastal lubricant base stock with sulfuric acid to remove colored bodies, aromatics and the like. A blend containing Product B in this oil was also tested. The bearing corrosion life of the base oil per se and of each of the blends is given in Table VI, below:

TABLE VI

| Product in Base Oil      | Bearing Corrosion Life (Hours) |
|--------------------------|--------------------------------|
| None (base oil alone) .. | 6                              |
| B ..                     | 10                             |
| C ..                     | 9                              |
| D ..                     | 13                             |
| E ..                     | 9                              |
| F ..                     | 9                              |
| G ..                     | 9                              |

All of the products improved the ability of the base oil to resist corrosion. The P<sub>2</sub>S<sub>5</sub>-treated C<sub>16</sub> "Oxo" ester of C<sub>10</sub>-C<sub>12</sub> alkenyl succinic acid was particularly effective.

The products of the present invention may be employed not only in ordinary hydrocarbon lubricating oils but also in the "heavy duty" type of lubricating oils which have been compounded with such detergent type additives as metal soaps, metal petroleum sulfonates, metal phenates, metal alcoholates, metal alkyl phenol sulfides, metal organo phosphates, phosphites, thiophosphates and thiophosphites, guanidine salts, metal xanthates and thioxanthates, metal thiocarbamates, and the like. Other types of additives, such as phenols and phenol sulfides, may also be present.

The lubricating oil base stocks used in the compositions of this invention may be straight mineral lubricating oils or distillates derived from paraffinic, naphthenic, asphaltic or mixed base crudes, or, if desired, various blended oils may be employed as well as residuals, particularly those from which asphaltic constituents have been carefully removed. Hydrogenated oils or white oils may be employed. Synthetic oils such as the polyether and polyester types or those prepared, for example, by the polymerization of olefins or by the reaction of oxides of carbon with hydrogen or by the hydrogenation of coal or its products may be used as such or in combination with each other and/or with mineral base lubricants. In certain instances cracking coil tar fractions and coal tar or shale oil distillates may also be used.

## 8

The additives are normally sufficiently soluble in the lubricant base stock, but in some cases auxiliary solvent agents may be used. The lubricating oils will usually range from about 40 to 150 seconds (Saybolt) viscosity at 210° F. The viscosity index may range from 0 to 100 or even higher.

Other agents than those which have been mentioned may be present in the oil composition, such as dyes, pour point depressants, heat thickened fatty oils, sulfurized fatty oils, sludge dispersers, anti-oxidants, thickeners, viscosity index improvers, oiliness agents, resins, rubber, olefin polymers, and the like.

What is claimed is:

1. As a new composition of matter a reaction product selected from the class consisting of: (A) the reaction products obtained by reacting, at a temperature in the range of about 200° to about 500° F. a reactive sulfur and phosphorus-containing material with an ester of an alkenyl succinic acid of the formula



in which R is an alkenyl radical having 4 to 24 carbon atoms, R' is selected from the group consisting of alkyl and alkenyl radicals having in the range of 1 to 30 carbon atoms, M is selected from the group consisting of R', a group I and II metal, and hydrogen and n is 1 to 2, and (B) metal salts of said reaction products and a group I and group II metal.

2. A composition as in claim 1 wherein said sulfur and phosphorus-containing material is a sulfide of phosphorus.

3. A composition as in claim 2 in which in the range of 0.2 to 1.5 mols of said sulfide of phosphorus per mol of said ester are reacted at a temperature in the range of about 250° to 450° F. for 1 to 10 hours.

4. A composition as in claim 3 wherein M is barium.

5. The process for producing a phosphorus and sulfur containing material which includes the steps of reacting together a compound selected from the group consisting of the esters of C<sub>4</sub> to C<sub>24</sub> alkenyl succinic acids and C<sub>1</sub> to C<sub>30</sub> aliphatic alcohols and the group I and group II metal salts of the partial esters of said succinic acids, and a sulfide of phosphorus at a temperature in the range of about 200° to 500° F.

6. A process as in claim 5 wherein said sulfide of phosphorus is phosphorus pentasulfide.

7. A process as in claim 6 wherein said reaction is carried out in the presence of an organic solvent.

8. A composition as in claim 1 wherein said R' group has in the range of 6 to 20 carbon atoms.

9. A composition as in claim 8 wherein said R' group has in the range of 6 to 16 carbon atoms.

10. As a new composition of matter, the product of the process of claim 5.

11. A process as in claim 5 in which said phosphorus and sulfur-containing material is further reacted with a metallic basic reacting compound, in which the metal is selected from groups I and II of the periodic table, to form a metal derivative thereof.

12. The process which comprises the steps of reacting the barium salt of an ester of aliphatic alcohol having 6 to 20 carbon atoms and a C<sub>6</sub>-C<sub>16</sub> alkenyl succinic acid with phosphorus pentasulfide at a temperature in the range of about 250° to 400° F.

13. A process as in claim 12 wherein said alkenyl succinic acid is a C<sub>10</sub>-C<sub>12</sub> alkenyl succinic acid.

14. The process which comprises the steps of reacting together an ester of an aliphatic alcohol having 6 to 20 carbon atoms and a C<sub>6</sub>-C<sub>16</sub> alkenyl succinic acid with

phosphorus pentasulfide at a temperature in the range of about 250° to 400° F.

15. As a new composition of matter, the product of the process of claim 12.

16. As a new composition of matter, the product of the 5 process of claim 14.

References Cited in the file of this patent

UNITED STATES PATENTS

|           |         |               |
|-----------|---------|---------------|
| 2,398,429 | Hughes  | Apr. 16, 1946 |
| 2,454,862 | Collins | Nov. 30, 1948 |
| 2,489,249 | Adelson | Nov. 29, 1949 |
| 2,516,119 | Hersh   | July 25, 1950 |